# EUROPEAN PATENT SPECIFICATION

(11) **EP 0 150 226 B1**
(45) Date of publication and mention of the grant of the patent: **04.11.1987**
(21) Application number: 83113078.6
(22) Date of filing: 23.12.1983
(51) Int. Cl.: B22D 27/00, B22D 1/00, B22D 21/02, B22D 5/04

(54) **Process and apparatus for minimizing foam formation during free falling of molten metal into moulds, launders or other containers**
Verfahren und Vorrichtung zur Vermeidung von Schaumformung beim freifallenden Giessstrahl in Giessformen, Giessrinnen oder andere Gefässe
Procédé et installation pour minimiser la formation d'écume pendant la chute libre du métal liquide dans les moules, goulottes ou autres récipients

(43) Date of publication of application: 07.08.1985
(73) Proprietor: NORANDA INC., Toronto Ontario, M5L 1B6 (CA)
(72) Inventor: Gervais, Edouard, Montreal Quebec, H3L 2W1 (CA); Levert, Henri, Lachine Quebec, H8S 4C5 (CA); Smyth, Laurence C., Beaconsfield Quebec, H9W 1R8 (CA); Deep, George, Pointe Claire Quebec, H9R 1M4 (CA)
(74) Representative: Müller-Boré & Partner Patentanwälte

## Description

This invention relates to a process for minimizing foam formation on the top surface of molten metal during pouring of the metal into moulds or similar containers, or during free falling of molten metal from a furnace to a launder, or cascading of the metal from launder to launder.

During pouring of free falling of molten metal, such as zinc, a considerable amount of foamed metal is formed on the top surface of the molten metal. This foam is normally skimmed off the surface of the molten metal manually. The task is arduous, requires workers to be in close proximity to molten metal and produces significant amounts of foamed metal which must be reclaimed.

Experiments carried out by the applicant during pouring of molten zinc into moulds have revealed that the formation of foam was due to the entrainment of air by the falling stream of molten metal. Hence air is transported below the molten metal surface to form air bubbles within the molten metal. Due to oxidation, a thin but tenacious zinc oxide film is formed on the inside surfaces of the bubbles. These bubbles rise to the surface and, as they emerge at the surface, it is observed that the outer surface of the bubbles is also oxidized and, in the case of large bubbles (approximately 12.5 mm diameter), that part of the upper skin of the bubble may freeze immediately although the metal pool beneath it remained liquid for several minutes longer.

Having realized that the foam formed on top of the molten metal is due to the formation of a zinc oxide film on the surface of the bubbles, applicant investigated several methods by which the bubbles could be either released or prevented from forming. As a result of such investigation, applicant has discovered that foam formation may be minimized by maintaining the molten metal, during filling of the mould, or free failing of the molten metal into launders or other containers, under an essentially non-oxidizing atmosphere so as to prevent entrainment of sufficient oxygen into the molten metal by the falling stream to form an excessive amount of bubbles having a tenacious oxidized film and which do not collapse when they float to the surface of the molten metal but rather produce undesirable foam on such surface.

The non-oxidizing atmosphere is preferably provided by an inert gas, such as nitrogen, and it can contain a small quantity of oxygen, e.g. up to 2% without producing excessive quantities of bubbles.

The above disclosed method may be carried out by placing a cover on the top of the molten metal container, and by providing an aperture therein for passage of the molten metal and means for introducing a non-oxidizing gas under the cover.

The above disclosed method could also be carried out on a continuous slab casting machine comprising a train of closely spaced open top ingot moulds mounted on an endless conveyor chain by providing a hood over the casting machine at the filling station and introducing a non-oxidizing gas under the hood. Seals would be required at the hood entrance and exit as well as on the sides to prevent excessive loss of non-oxidizing gas. The hood would of course require a sealed opening for introducing the molten metal through one of the walls thereof.

The above disclosed method could additionally be carried out on a continuous slab casting machine by an apparatus as disclosed in EP-A-0,088,701 which comprises a hood or a cover located at a small distance above the travelling moulds and adapted to cover two adjacent moulds. The cover has an opening in the top thereof for introducing molten into the moulds as well as an opening in the side for introducing a non-oxidizing under the cover. However, this apparatus does not allow an adequate distribution of the non-oxidizing gas in the moulds.

The apparatus in accordance with the present invention comprises a cover plate located at a predetermined distance above a number of containers or ingot moulds and having an aperture therein for casting molten metal in each container as they pass under the aperture. The cover plate extends over several moulds located before and several moulds located after said aperture and has a plurality of ports longitudinally spaced therein and over each mould for feeding a non-oxidizing gas through the cover plate so as to progressively develop a non-oxidizing atmosphere in the moulds as they approach the aperture in the cover plate and to maintain such atmosphere in the moulds as they pass beyond said aperture.

The entrance length of the cover plate before the mould filling aperture is necessary to progressively develop the required non-oxidizing atmosphere while the exit length of the cover plate is needed to maintain the required non-oxidizing atmosphere. The entrance length is determined by the conveyor line speed, the container volume, the container to cover gap and the influence of these factors on the volume of purging gas required to obtain the desired atmosphere. The exit length is determined by the pneumatic resistance required to prevent back flow of air into the container being filled.

At a conveyor line speed of 5 cm/sec. and with 25.5 kg ingot moulds, it has been found that oxygen levels less than 0.5% can be achieved with gaps up to 7.6 mm and gas flowrates lower than 56.6 Nm³h using a plate having a length equal to the width of five moulds (three before and two after the mould filling aperture).

The invention will now be disclosed by way of example with reference to the accompanying drawings in which:
Figure 1 is an apparatus used to carry out laboratory experiments with a fixed slab mould;
Figure 2 is an example of an apparatus used in the casting of molten metal into discrete moulds on a continuous ingot moulding machine;
Figure 3 is a view taken along line 3-3 of Figure 2;
Figure 4 is a view taken along line 4-4 of Figure 2;
Figure 5 is a graph illustrating the effect of varying gap dimension on oxygen level in mould atmosphere for a fixed nitrogen consumption;
Figure 6 is a graph illustrating the effect of varying nitrogen consumption on oxygen level in mould atmosphere for two different gap dimensions;
Figures 7 and 8 show mould refinements to reduce the gas flow requirement; and
Figure 9 shows another possible refinement which reduces gas flow but involves a non rubbing seal.

Referring to Figure 1, the laboratory apparatus comprises a bottom-pouring tundish 10 which is used to feed molten zinc into a slab mould 12 through a cover 14 closing the top of the mould. The bottom of the tundish is provided with an opening registering with a corresponding opening in the cover 14 and is sealed to the cover by any suitable means such as by welding. The opening in the bottom of the tundish is closed by a plug valve 16 which may be opened when it is desired to pour molten metal into the mould. The cover is sealed to the mould by '0' ring 18. A metered nitrogen inlet 20 and exhaust vent 22 are provided through the cover to maintain a suitable non-oxidizing atmosphere on the top surface of the mould.

A preliminary experimental procedure was carried out involving filling the tundish with molten zinc and then opening the valve to fill the mould. A fair amount of foam was formed on the top of the molten metal. The same procedure was repeated except that the covered mould was purged with nitrogen before opening the valve to fill the mould. The mould was uncovered soon after filling, before solidification to allow freezing of metal in air. No foam appeared on top of the molten metal.

A series of casting trials were carried out while varying the metal casting temperature and the concentration of oxygen in nitrogen. The effects of varying metal casting temperature were . observed in the normal zinc casting temperature range of 440-530°C. Purging was carried out at gas flow rates of 20 I/min. for one minute with nitrogen atmospheres ranging from commercial purity to concentrations of 2% oxygen. Foam-free surfaces on slab ingots were obtained with concentrations of oxygen in nitrogen varying from 0 to about 2%. It was also observed that the effects of temperature and oxygen are interactive as far as the production of acceptable slab surfaces is concerned. The conditions which produce acceptable surfaces on slab ingots are summarized below:
(a) Commercially-pure nitrogen atmosphere at temperatures less than 450°C. These conditions produce a brilliant, crystalline surface which is visible through a fully transparent oxide film. At temperatures higher than 450°C the phenomenon commonly referred to as "colouration" in which colours ranging from straw to dark purple was observed.
(b) Oxygen concentrations of approximately 2% at temperatures in the range of 450-4.75°C. These conditions result in a smooth silvery oxide film at the ingot surface.

The invention may also be carried out on a continuous slab casting machine, such as the Sheppard casting machine which has a number of moulds mounted on an endless conveyor chain. On such machines, the non-oxidizing atmosphere may be provided by means of a hood surrounding the casting machine at the filling station. Molten metal would be fed from the furnace to a pouring ladle located inside the hood and from the pouring ladle into the moulds as they move past the filling station. A metered nitrogen inlet and exhaust vent would be provided through the hood to provide a non-oxidizing atmosphere in the hood. The nitrogen atmosphere within the hood must be maintained at a slight positive pressure such that the ambient oxidizing atmosphere outside the hood cannot enter the hood through the mould entrance and exit ports. However, seals would be required at the hood entrance and exit to prevent excessive loss of nitrogen gas.

Referring to Figure 2, there is shown a train of closely spaced open top ingot moulds 30 mounted on an endless conveyor chain 32 moving at a line speed of about 5 cm/sec. in the direction indicated by arrow A. The ingot moulds all have flat top surfaces. A stationary cover plate 34 is mounted adjacent to but spaced by a predetermined distance D from the top surface of the moulds and covers a predetermined number of moulds before and after a metal pouring station which is mounted on the top of the cover plate. The metal pouring station is a conventional design comprising a launder 36 which ends with a downspout 38 used to feed molten metal into a ladle 40. The ladle 40 is intermittently pivoted to successively pour metal into each mould through a pouring slot 42 in the cover plate. A trap 44 is positioned at the end of the launder to capture dross which may be floating on the surface of the molten metal.

As shown in Figure 3, the cover plate 34 is provided with a predetermined number of gas inlet ports 46 and an inert gas is fed into such ports through a front manifold 48 and a main manifold 50. Inert gas is fed to the front mould entering under the plate through three gas inlet ports to rapidly purge the moulds, and to the remaining moulds under the plate through a single row of ports to progressively lower and maintain the oxygen level at the pouring station below a predetermined value. An auxiliary manifold 52 is also provided for feeding inert gas to the ladle enclosure 54 and the downspout enclosure 56. Cover strips 58 are placed on the gaps between the moulds so as to prevent excessive leakage of gas through such gaps.

As shown in Figure 4, the width of the plate 34 is equal to that of moulds 30. Inert gas enters the moulds at gas ports 46 and flows out through the gaps at the sides and the ends of the cover plate. The width of the cover as well as the width of the container with respect to the container cavity are dependent on the pneumatic resistance required to prevent back flow of air into the moulds.

It has been found that by controlling the length of the cover plate 34, the number and location of gas emission ports, the gas flow rate and the gap between the moulds and the cover plate, a desired inert atmosphere can be maintained below the pouring slot 42 without having to use contacting seals. To facilitate investigation of the gas inlet port spacing, gap dimension and inert gas (nitrogen) flow rate, an apparatus was designed in the laboratory to simulate a conventional casting machine. The number of gas inlet ports in the cover plate was set so that, at any time there was a minimum of three and a maximum of four gas parts above a traversing mould. The length of the cover plate was such that at any time five moulds (three before and two after pouring slot 22) were located under the cover plate.

The tests were carried out by establishing a predetermined nitrogen flow rate through the cover plate and then traversing the moulds past the cover plate at the same speed as a conventional casting machine conveyor (5 cm/sec.). Each mould was progressively purged as it entered under the cover plate. The mould atmosphere was sampled in the centre of the mould by pumping a sample to an oxygen analyser as the mould approached the pouring slot.

Experiments were carried out to determine the oxygen concentration in the mould atmosphere (a) at varying mould to cover gap dimensions and constant nitrogen flow rates and (b) at varying nitrogen flow rates and constant gap dimension. The results of these trials are presented in Figures 5 and 6. The front manifold flowrate in the test shown in Figure 5 was about 5.7 Nm³h and the main manifold flow rate was about 42.5 Nm³h. In the test shown in Figure 6, the front manifold flowrate was fixed at about 5.7 Nm'h and the main manifold flowrate was varied from 14.2 to 85 Nm^{Z}h.

The results of these tests presented in Figure 5 revealed that the oxygen level increased very rapidly for gap dimensions greater than 6.35 mm. More importantly, this curve illustrates that less than 0.5% oxygen can be achieved with gaps up to 7.62 mm with economically feasible gas consumption (-56.7 Nm³h). The effect of varying nitrogen consumption on the oxygen level in the mould atmosphere is illustrated in Figure 6 for two different gap dimensions of 2.5 and 3.2 mm. From these curves, it is evident that no gain is achieved by increasing atmosphere usage beyond 56.7 Nm³h and that acceptable oxygen levels are easily obtained with very low (28.3 Nm³h) gas consumption. The gap heights of 2.5 and 3.2 mm. used in these tests are practical values which can be achieved and maintained on present casting machines. Closer tolerances, which should be aimed for in the design of future casting machines can result in less than 0.1% oxygen with economical usage.

Following completion of the above pilot plant tests, equipment such as shown in Figure 2 was installed on a slab ingot casting machine at Canadian Electrolytic Zinc Limited, Valleyfield, Quebec, Canada to demonstrate, under plant production conditions, that skimming-free slabs can be produced by pouring liquid zinc in a nitrogen atmosphere.

Atmosphere tests were initially carried out with the machine in operation but without pouring liquid metal. These tests indicated that oxygen levels could be maintained at the pouring station in the range of 0.3-0.5% and that no gain could be achieved by increasing the nitrogen flow rate above 56.7 Nm³h.

Liquid zinc was then started up with preheating flames on the launder and ladle. Nitrogen was first delivered at 7.1 Nm³h to the front manifold and at 42.5 Nm³h to the main manifold of the cover plate and successively to the ladle and downspout enclosures at 7.1 Nm³h. The oxygen level maintained at the pouring station was in the range of 0.35-0.45%.

Major reduction in the foam floating on cast slabs was observed even before start-up procedures were completed. Total absence of foam was achieved when the closure and purging of the ladle and launder enclosures were completed.

The slab ingot surfaces were seen to be bright and dross-free. Transparent oxide films identical to those obtained in the laboratory tests using oxygen levels in the range of 0.2-0.5% were observed on the slabs.

Figures 7, 8 and 9 show refinements to reduce loss of gas in between the moulds and so reduce the gas flow requirements. In Figure 7, the edges of the moulds are thicker than that shown in Figure 2 and this increases the resistance to gas flow in the gap 60 between the moulds. In Figure 8, the edges of the moulds are designed so that the gap 62 is horizontal in order to prevent direct flow of the gas from the cover ports. This design is in a way equivalent to the cover strips 58 of Figure 2 but is much more resistant to wear and tear. Figure 9 shows another method of reducing gas flow which involves the use of a seal 64 in between the moulds. This alternative is possible since this seal is non rubbing.

## Claims

1. An apparatus for use on a continuous casting machine having a train of closely spaced open top moulds (30) mounted on an endless conveyor (32), comprising a cover plate (34) located at a predetermined distance above a number of said moulds (30) and having an aperture (42) therein for casting molten metal in each mould (30) as they pass under the aperture (42), and means (48, 50) for feeding a non-oxidizing gas into the moulds (30) under the cover, characterized in that, said cover plate (34) extends over several moulds (30) located before and several moulds (30) located after said aperture (42) and has a plurality of ports (46) longitudinally spaced therein and over each mould (30) for feeding a non-oxidizing gas through the cover plate (34) so as to progressively develop a non-oxidizing atmosphere in the moulds (30) as they approach the aperture (42) in the cover plate (34) and to maintain said atmosphere in the moulds (30) as they pass beyond said aperture (42).

2. An apparatus as defined in claim 1, wherein said atmosphere is an inert atmosphere.

3. An apparatus as defined in claim 1, further comprising sealing means (58) disposed across the gaps between said open top moulds (30), thereby preventing excessive leakage of gas through said gaps.

4. An apparatus as defined in claim 1, further comprising a metal pouring station for casting said molten metal in each mould (30) through the aperture (42) in said cover plate (34).

5. An apparatus as defined in claim 4 wherein said metal pouring station includes the end of a launder (36) which is provided with a downspout (38) used to feed molten metal into a ladle (40) which is intermittently pivoted to successively pour molten metal into each mould (30).

6. An apparatus as defined in claim 5, further comprising means (44) positioned at the end of the launder (32) to capture dross which may be floating on the surface of the molten metal.

7. An apparatus as defined in claim 5, further comprising an enclosure (54) around said ladle (40), said downspout (38) and the aperture (42) in said plate (34), and means (52) for feeding a non-oxidizing gas into said enclosure (54).

## Patentansprüche

1. Vorrichtung zur Verwendung an einer kontinuierlichen Gießmaschine mit einer Kette von in nahem Abstand angeordneten oben offen Formen (30), die auf einem endlosen Förderband (32) angeordnet sind, umfassend eine Abdeckplatte (34), die in einem vorbestimmten Abstand über einer Anzahl dieser Formen (30) angeordnet ist und eine Öffnung (42) darin für das Giessen von schmelzflüssigem Metall in jede Form (30) aufweist, während sie unter der Öffnung (42) durchgeht und Mittel (48, 50) für die Zufuhr eines nicht oxidierenden Gases in die Formen (30) unter der Abdeckung, dadurch gekennzeichnet, daß die Abdeckplatte (34) sich über mehrere Formen (30), die vor, und mehrere Formen (30), die nach dieser Öffnung (42) angeordnet sind, erstreckt und eine Mehrzahl von Durchgängen (46) hat, die in Längsrichtung im Abstand voneinander darin und über jeder Form (30) angeordnet sind, so daß nach und nach eine nicht oxidierende Atmosphäre in den Formen (30) ausgebildet wird, während sie sich der Öffnung (42) in der Abdeckplatte (34) nähern und diese Atmosphäre in den Formen (30) aufrechterhalten wird, während sie unter der Öffnung (42) durchgehen.

2. Vorrichtung nach Anspruch 1, dadurch gekennzeichnet, daß die Atmosphäre eine inerte Atmosphäre ist.

3. Vorrichtung nach Anspruch 1, dadurch gekennzeichnet, daß sie weiter Dichtmittel (58) aufweist, die quer über die Spalte zwischen den oben offenen Formen (30) angeordnet sind und dadurch einen übermäßigen Austritt von Gas durch diese Spalte verhindern.

4. Vorrichtung nach Anspruch 1, dadurch gekennzeichnet, daß sie weiterhin eine Metallgießstation zum Giessen des schmelzflüssigen Metalls in jede Form (30) durch die Öffnung (42) in dieser Abdeckplatte (34) enthält.

5. Vorrichtung nach Anspruch 4, dadurch gekennzeichnet, daß die Metallgießstation das Ende einer Gießrinne (36) umfaßt, die mit einem Auslauf (38) versehen ist, der zum Zuführen des schmelzflüssigen Metalls in einen Gießlöffel (40) dient, welcher intermittierend gedreht wird, um nacheinander schmelzflüssiges Metall in jede Form (30) zu gießen.

6. Vorrichtung nach Anspruch 5, dadurch gekennzeichnet, daß sie weiter Mittel (44) enthält, die am Ende der Gießrinne (36) angeordnet sind, um Krätze abzufangen, die auf der Oberfläche des schmelzflüssigen Metalls schwimmen kann.

7. Vorrichtung nach Anspruch 5, dadurch gekennzeichnet, daß sie weiter ein Gehäuse (54) um die Gießpfanne (40), den Auslauf (38) und die Öffnung (42) in der Platte (34) enthält und Mittel (52) für die Zufuhr eines nicht oxidierenden Gases in dieses Gehäuse (54).

## Revendications

1. Un dispositif destiné à être utilisé sur une machine de coulée continue comportant un train de moules (30) ouverts à la partie supérieure et rapprochés les uns des autres montés sur un transporteur sans fin (32), comprenant une plaque de recouvrement (34) disposée à une distance prédéterminée au-dessus de certains desdits moules (30) et ayant une ouverture (42) pour le métal fondu coulé dans chaque moule (30) lorsqu'il passe sous l'ouverture (42) et des moyens (48, 50) pour fournir un gaz non oxydant à l'intérieur des moules (30) sous la plaque de recouvrement, caractérisé en ce que, ladite plaque de recouvrement (24) s'étend sur plusieurs moules (30) disposés avant et plusieurs moules (30) disposés après ladite ouverture (42) et présente une pluralité d'orifices (46) espacées longitudinalement et au-dessus de chaque moule (30) pour fournir un gaz non oxydant à travers la plaque de recouvrement (34) de manière à développer progressivement une atmosphère non oxydante dans les moules (30) lorsqu'ils s'approchent de l'ouverture (42) dans la plaque de recouvrement (34) et pour maintenir ladite atmosphère dans les moules (30) lorsqu'ils dépassent ladite ouverture (42).

2. Dispositif selon la revendication 1, dans lequel ladite atmosphère est une atmosphère inerte.

3. Un dispositif selon la revendication 1, comportant en outre des moyens de fermeture étanches (58) disposés dans les intervalles ménagés entre lesdits moules (30) ouverts ù la partie supérieure de manière à empêcher la fuite excessive de gaz à travers lesdits intervalles.

4. Un dispositif selon la revendication 1, comprenant en outre un poste de coulée du métal pour couler ledit métal fondu dans chacun des moules (30) à travers l'ouverture (42) ménagée dans ladite plaque de recouvrement (34).

5. Un dispositif selon la revendication 4, dans lequel ledit poste de coulée du métal comprend l'extrémité d'un chenal de coulée (36) qui est muni d'une goulotte (38) utilisé pour fournir le métal fondu dans une poche (40) qui pivote de façon intermittente pour verser successivement le métal fondu dans chaque moule (30).

6. Un dispositif selon la revendication 5, comportant en outre des moyens (44) disposés à l'extrémité du chenal de coulée (36) pour recueillir les crasses qui peuvent flotter sur la surface du métal fondu.

7. Un dispositif selon la revendication 5, comportant en outre une enceinte (54) autour de ladite poche (40) ladite goulotte (38) et l'ouverture (42) ménagées dans ladite plaque (34) et des moyens (52) pour fournir un gaz non oxydant à l'intérieur de ladite enceinte (54).
